# EUROPEAN PATENT SPECIFICATION

(11) **EP 2 367 967 B1**
(45) Date of publication and mention of the grant of the patent: **31.08.2016**
(21) Application number: 10825829.4
(22) Date of filing: 19.07.2010
(51) Int. Cl.: C23C 18/24, G03F 7/004, H05K 3/10, C23C 18/16, C23C 18/18, C23C 18/31, C25D 5/56

(54) **SURFACE METALIZING METHOD, METHOD FOR PREPARING PLASTIC ARTICLE AND PLASTIC ARTICLE MADE THEREFROM**
OBERFLÄCHENMETALLISIERUNGSVERFAHREN, VERFAHREN ZUR HERSTELLUNG EINES KUNSTSTOFFARTIKELS UND DARAUS HERGESTELLTER KUNSTSTOFFARTIKEL
PROCÉDÉS DE MÉTALLISATION DE SURFACE, DE PRÉPARATION D'ARTICLE EN PLASTIQUE ET ARTICLE EN PLASTIQUE FABRIQUÉ PAR CE PROCÉDÉ

(30) Priority: 15.01.2010 CN 201010044447
(43) Date of publication of application: 28.09.2011
(73) Proprietor: BYD Company Limited, Shenzhen 518118 (CN); Shenzhen BYD Auto R&D Company Limited, Shenzhen, Guangdong 518118 (CN)
(72) Inventor: GONG, Qing, Shenzhen Guangdong 518118 (CN); MIAO, Weifeng, Shenzhen Guangdong 518118 (CN); ZHOU, Liang, Shenzhen Guangdong 518118 (CN); ZHANG, Xiong, Shenzhen Guangdong 518118 (CN)
(74) Representative: Gulde & Partner
(86) International application number: PCT/CN2010/075232
(87) International publication number: WO 2011/085584

(56) References cited:
- EP-A1- 1 274 288
- EP-A1- 1 650 249
- CN-A- 1 518 850
- CN-A- 1 542 547
- CN-A- 101 394 710
- JP-B- 58 018 932
- RU-C1- 2 192 715
- RU-C2- 2 188 879
- US-A1- 2003 031 803
- US-A1- 2003 134 558
- US-A1- 2006 286 365

## Description

The present disclosure relates to surface treatment, more particularly to surface metallization on non-metal material such as plastic, i.e. surface metalizing method and a plastic article made therefrom.

### BACKGROUND

Plastic substrates having a metalized layer on their surfaces as pathways of electromagnetic signal conduction are widely used in automobiles, industries, computers and telecommunications etc. Selectively forming a metalized layer is one of the important processes for preparing such plastic products. The method for forming a metalized layer in prior art is usually practiced by forming a metal core as a catalytic center on the plastic support surface so that chemical plating may be performed. However, processes related thereto are complex where strict demand on equipment is needed whereas the energy consumption is high. Further, there is a low adhesive force between the coating and the plastic support.

### SUMMARY

In viewing thereof, there remains an opportunity to provide a method for metalizing a plastic surface, in which the plastic metallization is easily performed with lower energy consumption and enhanced adhesive force between the coating layer and the plastic support. Further, there remains an opportunity to provide a method for preparing a plastic article and a plastic article made therefrom, in which the adhesive force between the coating layer and the plastic or non-metal support is enhanced.

According to an embodiment of the invention, a method for metalizing a plastic surface of a plastic article is provided. The plastic article having at least a part thereof made from a support comprising a supporting material and a chemical plating promoter. The method comprises the steps of: 1) gasifying the plastic surface to expose the chemical plating promoter; 2) chemical plating a layer of copper or nickel on the plastic surface; and 3) plating the plated surface in step 2) by electroplating or chemical plating at least one more time to form a metalized layer on the plastic surface. The chemical plating promoter is a perovskite-based compound represented by a general formula of ABO₃, in which A is one or more elements selected from groups 9, 10, and 11 of the periodic table and, optionally, one or more additional elements selected from groups 1 (IA), 2 (IIA), and the lanthanide series of the periodic table, and B is one or more elements selected from groups 4 (IVB) and 5 (VB) of the periodic table.

According to another embodiment of the invention, a plastic article made by the method as described above is provided.

As found by the inventors that, selectively chemical plating may be directly performed on the surface containing the chemical plating promoter, and the plastic will not be degraded by the perovskite-based compounds represented by a general formula of ABO₃ without reducing metal oxides into pure metals.

According to an embodiment of the disclosure, the chemical plating promoter may be a material selected from the group consisting of CaCu₃Ti₄O₁₂, Na_{0.04}Ca_{0.98}Cu₃Ti₄O₁₂, La_{0.01}Ca_{0.99}Cu₃Ti₄O₁₂, CuTiO₃, CuNiTi₂O₆, CuNbO₃, CuTaO₃, CuZrO₃ and any combination thereof.

The chemical plating promoter may be distributed evenly in the plastic support, and a predetermined area on the surface of the plastic support which may be gasified by, for example, laser to expose the chemical plating promoter so that the chemical plating promoter may not be reduced into pure metal without high energy consumption. And further electroplating or chemical plating may be performed to form the desired metalized layer, thus achieving the selective surface metallization with simple process, lower energy consumption and reduced cost.

In addition, the chemical plating promoter may be evenly distributed in the plastic support, so that the adhesive force between the coating layer and the plastic support after chemical plating is high, thus improving the quality of the plastic article as manufactured therefrom.

Additional aspects and advantages of the embodiments of present disclosure will be given in part in the following descriptions, become apparent in part from the following descriptions, or be learned from the practice of the embodiments of the present disclosure.

### DETAILED DISCRIPTION OF THE EMBODIMENT

Reference will be made in detail to embodiments of the present disclosure.

The embodiments described herein are explanatory, illustrative, and used to generally understand the present disclosure. The same or similar elements and the elements having same or similar functions are denoted by like reference numerals throughout the descriptions.

In the following, a method for metalizing a plastic surface is provided. The plastic comprises a support or supporting material and a chemical plating promoter. According to an embodiment of the disclosure, the method comprises the steps of: 1) gasifying the plastic surface to expose the chemical plating promoter; 2) chemical plating a layer of copper or nickel on the plastic surface, and 3) plating the plated surface in step 2) by electroplating or chemical plating at least one more time to form a metalizing layer on the plastic surface. The plastic surface may be gasified by laser to expose the chemical plating promoter. And the laser may have a wavelength ranging from about 157 nm to about 10.6 µm with a scanning speed from about 500 mm/s to about 8000 mm/s, a scanning step from about 3 µm to about 9 µm, a scan time delay from about 30 µs to 100 µs, a laser power from about 3 W to about 4 W, a frequency from about 30 KHz to about 40 KHz and a filled distance from about 10 µm to about 50 µm.

The chemical plating promoter may have an average diameter ranging from about 20 nm to about 100 µm, preferably from about 50 nm to about 10µm, more preferably from about 200 nm to about 4 µm.

The chemical plating promoter is a perovskite-based compound represented by a general formula of ABO₃, in which A is one or more elements selected from groups 9, 10, and 11 of the periodic table and optionally selected from groups IA and IIA, and lanthanide series of the periodic table, and B is one or more elements selected from groups IVB and VB of the periodic table. For example, element A of the composite oxide ABO₃ may be an element selected from the group consisting of Co, Rh, Ni, Pd, Cu, Ag and any combination thereof, and may optionally containing an element selected from the group consisting of Na, Ca, La, Ce and any combination thereof. Element B may be an element selected from the group consisting of Ti, Zr, Nb, V and any combination thereof. According to an embodiment of the disclosure, the composite oxide ABO₃ may be CaₓCu₄₋ₓTi₄O₁₂, Na_{0.04}Ca_{0.98}Cu₃Ti₄O₁₂, La_{0.01}Ca_{0.99}Cu₃Ti₄O₁₂, CuNiTi₂O₆, CuNbO₃, CuTaO₃ or CuZrO₃, where 0≤x≤4.

More preferably, the composite oxide ABO₃ may include, but not limited to, CaCu₃Ti₄O₁₂, Na_{0.04}Ca_{0.98}Cu₃Ti₄O₁₂, La_{0.01}Ca_{0.99}Cu₃Ti₄O₁₂, CuTiO₃, CuNiTi₂O₆, CuNbO₃, CuTaO₃ or CuZrO₃.

The support or supporting material may be a thermoplastic or a thermosetting resin. The thermoplastic includes a material selected from the group consisting of polyolefins, polycarbonates (PC), polyesters, polyamides, polyaromatic ethers, polyester-imides, polycarbonate/acrylonitrile-butadiene-styrene composite (PC/ABS), polyphenylene oxide (PPO), polyphenylene sulfide (PPS), polyimides (PI), polysulfones (PSU), poly (ether ether ketone) (PEEK), polybenzimidazole (PBI), liquid crystalline polymer (LCP) and any combination thereof. The polyolefins may be selected from polystyrene (PS), polypropylene (PP), polymethyl methacrylate (PMMA) or poly(acrylonitrile-butadiene-styrene) (ABS). The polyesters may be selected from polycyclohexylene dimethylene terephthalate (PCT), poly(diallyl isophthalate) (PDAIP), poly(diallyl phthalate) (PDAP), polybutylene naphthalate (PBN), Poly(ethylene terephthalate) (PET), or polybutylene terephthalate (PBT). The polyamides may be selected from polyhexamethylene adipamide (PA-66), poly(hexamethylene azelamide) (PA-69), polyhexamethylene succinamide (PA-64), poly(hexamethylene dodecanoamide) (PA-612), poly(hexamethylene sebacamide) (PA-610), poly(decametylene sebacamide) (PA-1010), polyundecanoamide (PA-11), polydodecanoamide (PA-12), polycapryllactam (PA-8), polyazelamide (PA-9), polycaprolactam (PA-6), poly(p-phenytene terephthalamide) (PPTA), poly-m-xylylene adipamide (MXD6), polyhexamethylene terephthalamide (PA6T), or poly(nonamethylene terephthalamide) (PA9T). The liquid crystalline polymer (LCP) may be a polymer comprising rigid chains and being capable of forming regions of highly ordered structure in the liquid phase. The thermosetting resin includes a material selected from the group consisting of phenolic resin, urea-formaldehyde resin, melamine-formaldehyde resin, epoxy resin, alkyd resin, polyurethane and any combination thereof.

In the surface metalizing method as described above, because the surface of the plastic support may be gasified by, for example, laser to expose the chemical plating promoter, the chemical plating promoter may not be reduced into pure metal without high energy consumption. And the adhesive force between the coating layer and the plastic support after chemical plating is very high, thus improving the process of selective surface metallization.

The method for metalizing a plastic surface may be used for manufacturing a plastic article, such as a shell of an electrical device, for example, a mobile phone, a laptop computer, a shell of a refrigerator, a lamp stand, a plastic container etc., where selective surface metalizing treatment may be desired.

And in the following, a method for preparing a plastic article will be described in detail.

The method for preparing a plastic article comprises the steps of: 1) forming a plastic article having at least a part thereof made from a support comprising a support and a chemical plating promoter; 2) gasifying a surface of the support to expose the chemical plating promoter; and 3) chemical plating a layer of copper or nickel on the surface followed by electroplating or chemical plating at least one more time, to form a metalized layer on the surface.

The chemical plating promoter is a perovskite-based compound represented by a general formula of ABO₃, in which A is one or more elements selected from groups 9, 10, and 11 of the periodic table and optionally selected from groups IA and IIA, and lanthanide series of the periodic table, and B is one or more elements selected from groups IVB and VB of the periodic table. For example, element A of the composite oxide ABO₃ may be an element selected from the group consisting of Co, Rh, Ni, Pd, Cu, Ag and any combination thereof, and may optionally containing an element selected from the group consisting of Na, Ca, La, Ce and any combination thereof. Element B may be an element selected from the group consisting of Ti, Zr, Nb, V and any combination thereof. According to an embodiment of the disclosure, the composite oxide ABO₃ may be CaxCu₄₋ₓTi₄O₁₂, Na_{0.04}Ca_{0.98}Cu₃Ti₄O₁₂, La_{0.01}Ca_{0.99}Cu₃Ti₄O₁₂, CuNiTi₂O₆, CuNbO₃, CuTaO₃ or CuZrO₃, where 0≤x≤4.

More preferably, the composite oxide ABO₃ may include, but not limited to, CaCu₃Ti₄O₁₂, Na_{0.04}Ca_{0.98}Cu₃Ti₄O₁₂, La_{0.01}Ca_{0.99}Cu₃Ti₄O₁₂, CuTiO₃, CuNiTi₂O₆, CuNbO₃, CuTaO₃ or CuZrO₃.

The perovskite-based compound is known in the art. The perovskite-based compound may be commercially available, which may be ball milled to obtain the required diameter, or the perovskite-based compound may be prepared by a method known in the art. For example, a process for preparing CaCu₃Ti₄O₁₂ may comprise the steps of: mixing high purity CaCO₃, CuO, and TiO₂ powders according to the stoichiometric proportion; ball milling the powders in distilled water for about 12 hours to form a mixture; after drying, calcining the mixture at a temperature of about 950°C for about 2 hours; ball milling again; after drying, granulating the dried powders with the agglomerant polyvinyl alcohol (PVA) to obtain particles; pressing the particles into circular sheets under the pressure of about 100 MPa; and sintering the circular sheets at a temperature of about 1100°C for about 6 hours to form the promoter accordingly. Similarly, by the process as described above, Na_{0.04}Ca_{0.98}Cu₃Ti₄O₁₂ may be prepared by high purity Na₂CO₃, CaCO₃, CuO and TiO₂ powders, and La_{0.01}Ca_{0.99}Cu₃Ti₄O₁₂ may be prepared by high purity La₂O₃, CaCO₃, CuO and TiO₂ powders.

It is shown by a lot of research that, except that pure Cu and Pd may be used as the nucleus or grain for chemical plating, nano-CuO can improve the chemical deposition speed of the metal atoms on plastic surface during chemical plating. However, nano-CuO may also cause the degradation of the plastic. By many experiments, it has been found by the inventors that the perovskite-based compound represented by a general formula of ABO₃ may be used for surface treatment, and such chemical plating promoters may promote the chemical deposition of chemical plating on their surfaces without causing the degradation of the plastic while remained in the support for a long time.

The support may be firstly provided, comprising a support and a chemical plating promoter. The chemical plating promoter may be evenly distributed in the support.

The support may be a thermoplastic or a thermosetting resin. The thermoplastic includes a material selected from the group consisting of polyolefins, polycarbonates (PC), polyesters, polyamides, polyaromatic ethers, polyester-imides, polycarbonate/acrylonitrile-butadiene-styrene composite (PC/ABS), polyphenylene oxide (PPO), polyphenylene sulfide (PPS), polyimides (PI), polysulfones (PSU), poly (ether ether ketone) (PEEK), polybenzimidazole (PBI), liquid crystalline polymer (LCP) and any combination thereof. The polyolefins may be selected from polystyrene (PS), polypropylene (PP), polymethyl methacrylate (PMMA) or poly(acrylonitrile-butadiene-styrene) (ABS). The polyesters may be selected from polycyclohexylene dimethylene terephthalate (PCT), poly(diallyl isophthalate) (PDAIP), poly(diallyl phthalate) (PDAP), polybutylene naphthalate (PBN), Poly(ethylene terephthalate) (PET), or polybutylene terephthalate (PBT). The polyamides may be selected from polyhexamethylene adipamide (PA-66), poly(hexamethylene azelamide) (PA-69), polyhexamethylene succinamide (PA-64), poly(hexamethylene dodecanoamide) (PA-612), poly(hexamethylene sebacamide) (PA-610), poly(decametylene sebacamide) (PA-1010), polyundecanoamide (PA-11), polydodecanoamide (PA-12), polycapryllactam (PA-8), polyazelamide (PA-9), polycaprolactam (PA-6), poly(p-phenytene terephthalamide) (PPTA), poly-m-xylylene adipamide (MXD6), polyhexamethylene terephthalamide (PA6T), or poly(nonamethylene terephthalamide) (PA9T). The liquid crystalline polymer (LCP) may be a polymer comprising rigid chains and being capable of forming regions of highly ordered structure in the liquid phase. The thermosetting resin includes a material selected from the group consisting of phenolic resin, urea-formaldehyde resin, melamine-formaldehyde resin, epoxy resin, alkyd resin, polyurethane and any combination thereof.

The method of forming the plastic article may be any known in the art, which may comprise the steps of: firstly, mixing the promoter and the support uniformly to obtain a mixture; then processing the mixture in a conventional plastic mixing machine, such as a banbury mixer, a single screw extruder, a twin screw extruder or a blender, by injection molding, blow molding, extruding or hot pressing, to form a support with a desired shape.

The amount of the chemical plating promoter may be about 1 wt% to about 40 wt% based on the weight of the support. According to another embodiment of the present disclosure, the amount of chemical plating promoter may be about 1 wt% to about 30 wt% based on the weight of the support. According to still another embodiment of the present disclosure, the amount of chemical plating promoter may range from about 2 wt% to about 15 wt%, based on the weight of the support.

The support may further comprise a material selected from the group consisting of inorganic filler, antioxidant, light stabilizer, lubricant and any combination thereof. The inorganic filler, antioxidant, light stabilizer and lubricant may be commercially available, and may be mixed with the support and the chemical plating promoter to form the support.

Based on the weight of the support, the amount of the antioxidant may be about 0.01 wt% to about 2 wt%; the amount of the light stabilizer may be about 0.01 wt% to about 2 wt%; the amount of the lubricant may be about 0.01 wt% to about 2 wt%; and the amount of the inorganic filler may be about 1 wt% to about 70 wt%.

The antioxidant may enhance the oxidation resistance of the support, and may be those known in the art, such as antioxidants 1098, 1076, 1010, or 168 available from Ciba Specialty Chemicals. The light stabilizer may enhance the light stability of the support, and may be those well known in the art, preferably a hindered amine light stabilizer, such as a light stabilizer 944 available from Ciba Specialty Chemicals.

The lubricant may enhance fluidity of the plastic so that the plastic support may be evenly mixed. It may include a material selected from the group consisting of methylpolysiloxane, ethylene/vinyl acetate wax (EVA wax), polyethylene wax, stearate and any combination thereof.

The inorganic filler may be selected from talcum powders, calcium carbonate, glass fiber, calcium silicate fiber, tin oxide or carbon black. The glass fiber may increase the etched depth of the support while being gasified by laser, which is favorable for the adhesion of Cu during chemical plating of Cu. The tin oxide, especially nano tin oxide, or carbon black may enhance the energy utilization rate of the laser. In some embodiments, the inorganic filler may be further selected from micro glass bead, calcium sulfate, barium sulfate, titanium dioxide, pearl powder, wollastonite, diatomite, kaolin, coal powders, argil, mica, oil shale ash, aluminum silicate, alumina, carbon fiber, silicon dioxide or zinc oxide. Preferably, the inorganic filler may not contain elements harmful to the environment and the human body, such as Cr.

The chemical plating promoter may be evenly distributed in the support, the adhesive force between the chemical plating promoter and the support is very high so that the following chemical plating may be performed on the surface of the chemical plating promoter directly. As a result, the adhesive force between the formed coating layer and the support may be increased tremendously.

The laser-gasifying may be performed on the surface of the plastic article where the part made of the plastic is gasified to expose the chemical plating promoter. According to an embodiment of the disclosure, the desired pattern may be formed on the surface of the support by the method of the present disclosure. The laser equipment may be a conventional infrared laser, for example a CO₂ laser marking system. The wavelength of the laser may be about 157 nm to about 10.6 µm, the scanning speed may be from about 500 mm/s to about 8000 mm/s, the scanning step size may be about 3 µm to about 9 µm, the scan time delay may be about 30 µs to about 100 µs, the laser power may be about 3 W to 4 W, the frequency may be from about 30 KHz to about 40 KHz, and the filled distance may be about 10 µm to about 50 µm. The energy demand of the present disclosure may be low, because it just needs to gasify the surface of the support to expose the chemical plating promoter, without reducing the support to the pure metal.

The thickness of the support may be greater than about 500 µm, and the etched depth of the support may be about 1 µm to about 20 µm, so that the chemical plating promoter may be exposed to form a microscopic and coarse surface having rugged voids. During the following process of chemical plating a copper or nickel layer, copper or nickel may be embedded into the voids of the coarse surface, thus forming strong adhesive force with the plastic support.

The gasifying of the plastic support may cause plastic smoke, which may drop down and cover the exposed chemical plating promoter. According to an embodiment of the disclosure, a ventilating unit may be used during laser-gasifying for exhausting the smoke. Additionally, the ultrasonic cleaning may be performed on the support after laser-gasifying.

The process of chemical plating a copper or nickel layer may be performed on the exposed chemical plating promoter, and then electroplating or chemical plating again to form a metalized layer area on the support. The chemical plating method may be any one practiced in the art. For example, the support may be immersed into a chemical plating bath.

After contacted with the chemical copper plating solution or chemical nickel plating solution in the chemical plating bath, the exposed chemical plating promoter may promote Cu ion or Ni ion to undertake reduction to form pure Cu or Ni particles which envelop the surface of the chemical plating promoter so that a compact or dense first plating layer may be formed on the laser-gasified area.

To increase surface decorativeness, applicability and corrosion resistance, one or more plating layers may be formed on the first plating layer to obtain the final metalized layer.

In one embodiment, the first plating layer may be a nickel layer, a second chemical plating may be performed on the nickel layer to form a second copper layer, and then a third chemical plating may be performed on the second layer to form a third nickel layer. As the result, the metalized layer may be of a Ni-Cu-Ni structure from the inside of the plastic article to the outside thereof. In another embodiment, an Au layer may be strike plated on the Ni-Cu-Ni layer to obtain a metalized layer of Ni-Cu-Ni-Au.

In another embodiment, the first plating layer may be a copper layer, and a second electroplating may be performed on the copper layer to form a second nickel layer. As the result, the metalized layer may be of a Cu-Ni structure from the inside of the plastic article to the outside thereof. In yet another embodiment, an Au layer may be strike plated on the Cu-Ni layer to obtain a metalized layer of Cu-Ni-Au.

In the metalizing layers of Ni-Cu-Ni, Ni-Cu-Ni-Au, Cu-Ni or Cu-Ni-Au, the thickness of the Ni layer may be about 0.1 µm to about 50 µm, preferably, about 1 µm to about 10 µm, more preferably, about 2 µm to about 3 µm; the thickness of the Cu layer may be about 0.1 µm to about 100 µm, preferably, about 1 µm to about 50 µm, more preferably, about 5 µm to about 30 µm; and the thickness of the Au layer may be about 0.01 µm to about 10 µm, preferably, about 0.01 µm to about 2 µm, more preferably, about 0.1 µm to about 1 µm.

The chemical copper and nickel plating solutions, the copper and nickel electroplating solutions and the aurum strike plating solution may be those known in the art or may be commercially available. According to an embodiment of the disclosure, the chemical copper plating solution having a pH value of from about 12 to about 13 may comprise a copper salt and a reducing agent which may reduce the copper salt to the metal copper and may be one or more compounds selected from glyoxylic acid, hydrazine and sodium hypophosphite. In one example, the chemical copper plating solution having a pH value of about 12.5 to about 13 adjusted by NaOH and H₂SO₄ may be proposed as follows: about 0.12 mol/L of CuSO₄·5H₂O, about 0.14 mol/L of Na₂EDTA-2H₂O, about 10 mg/L of potassium ferrocyanide, about 10 mg/L of 2, 2'-bipyridine, and about 0.10 mol/L of glyoxylic acid (HCOCOOH).

According to an embodiment of the disclosure, the chemical plating nickel solution having a pH value of about 5.2 adjusted by NaOH at a temperature of about 85-90°C may be proposed as follows: about 23 g/l of nickel sulfate, about 18 g/l of sodium hypophosphite, about 20 g/l of lactic acid, and about 15 g/l of malic acid.

The chemical plating copper time may be about 10 min to 240 min, and the chemical plating nickel time may be about 8 min to 15 min.

The aurum strike plating solution may be, for example, the neutral aurum plating solution BG-24 available from Jingyanchuang Chemical Company, Shenzhen, P. R. C.

There are substantially no chemical plating deposits on the surface of the support where no chemical plating promoters exist. Thus, the electroplating speed is very low with weak adhesive force. Even there are few chemical deposits, they may be removed easily. Thus, direct selective surface metalizing method may be achieved easily according to the present disclosure.

Further, the present disclosure discloses a plastic article as manufactured by the method as mentioned above. The plastic article may comprise a support and a metalized layer area on a surface of the support. The metalized layer may be a Ni-Cu-Ni layer, a Ni-Cu-Ni-Au layer, a Cu-Ni layer or a Cu-Ni-Au layer from the inner portion of the plastic article to the outer portion thereof.

Additional details of the present disclosure will be provided as follows by some embodiments of the present disclosure.

### Embodiment 1

A method for preparing a plastic article comprises the steps of:
a) ball milling CaCu₃Ti₄O₁₂ in a high speed ball grinder for about 10 hours to form powders with an average diameter of about 700 nm; mixing PPE/PPS resin alloy, CaCu₃Ti₄O₁₂ powders, calcium carbonate fiber, and antioxidant 1010 according to a weight ratio of about 100 : 10 : 30 : 0.2 in a high speed mixer to prepare a mixture; extruding and granulating the mixture by a twin screw extruder available from Nanjing Rubber & Plastics Machinery Plant Co., Ltd., P. R. C.; and injection molding the mixture to form a substrate of a circuit board for a LED (light emitting diode) lamp;
b)patterning on the substrate by a DPF-M12 infrared laser available from Shenzhen TEC-H LASER Technology Co., Ltd., P. R. C. with a wavelength of about 1064 nm, a scanning speed of about 1000 mm/s, a scanning step size of about 9 µm, a scan time delay of about 30 µs, a frequency of about 40 KHz, a power of about 3 W, and a filled distance of about 50 µm; ultrasonic cleaning the surface of the support; and
c) immersing the substrate in a chemical nickel plating solution for about 10 min to form a first nickel layer with a thickness of about 3 µm; immersing the substrate in a chemical copper plating solution for about 4 hours to form a copper layer with a thickness of about 13 µm on the first nickel layer; immersing the substrate in the chemical nickel plating solution for about 10 min again to form a second nickel layer with a thickness of about 3 µm on the copper layer; and strike plating an aurum layer with a thickness of about 0.03 µm on the second nickel layer to form the plastic article as the substrate for a circuit board of a LED lamp; where the nickel plating solution was comprised of about 0.12 mol/L of CuSO₄·5H₂O, about 0.14 mol/L of Na₂EDTA·2H₂O, about 10 mg/L of potassium ferrocyanide, about 10 mg/L of 2,2'-bipyridine, and about 0.10 mol/L of glyoxylic acid (HCOCOOH), with a PH value of about 12.5 to about 13 adjusted by NaOH and H₂SO₄; the nickel plating solution was comprised of about 23 g/L of nickel sulfate, about 18 g/L of sodium hypophosphite, about 20 g/L of lactic acid, about 15 g/L of malic acid, with a PH value of about 5.2 adjusted by NaOH; and the aurum strike plating solution was BG-24 neutral aurum plating solution commercially available from Shenzhen Jingyanchuang Chemical Company, P. R. C.

### Embodiment 2

The method in Embodiment 2 is substantially similar in all respects to that in Embodiment 1, with the exception of:
in step a), ball milling CuNiTi₂O₆ to form powders with an average diameter of about 800 nm; drying the powders; mixing PEEK resin, CuNiTi₂O₆, glass fiber, and antioxidant 168 according to a weight ratio of about 100 : 20 : 30 : 0.2 in a high speed ball grinder to prepare a mixture; extruding and granulating the mixture; injection molding the mixture to form a shell; and
in step c), immersing the shell in a chemical nickel plating solution for about 8 min to form a nickel layer with a thickness of about 2 µm; immersing the shell in a chemical copper plating bath for about 3 hours to form a copper layer with a thickness of about 13 µm on the first nickel layer; immersing the shell in the chemical nickel plating solution for about 10 min again to form a second nickel layer with a thickness of about 3 µm on the copper layer; and strike plating an aurum layer with a thickness of about 0.03 µm on the second nickel layer to form the plastic article as a shell for an electronic connector shell of an automobile motor.

### Embodiment 3

The method in Embodiment 3 is substantially similar in all respects to that in Embodiment 1, with the exception of:
in step a), ball milling CuNbO₃ to form powders with an average diameter of about 800 nm; drying the powders; mixing PES resin, CuNbO₃, potassium titanate whisker, antioxidant 1010, and polyethylene wax according to a weight ratio of about 100 : 10 : 30 : 0.2 : 0.1 in a high speed ball grinder to prepare a mixture; extruding and granulating the mixture; injection molding the mixture to form a shell; and
in step c), immersing the shell in a chemical copper plating solution for about 3 hours to form a copper layer with a thickness of about 5 µm; and immersing the support in a chemical nickel plating solution for about 10 min to form a nickel layer with a thickness of about 3 µm on the copper layer, thus forming the plastic article as a shell for an electronic connector.

### Embodiment 4

The method in Embodiment 4 is substantially similar in all respects to that in Embodiment 1, with the exception of:
in step a), ball milling CuTiO₃ to form powders with an average diameter of about 900 nm; drying the powders; mixing PC resin, CuTiO₃, antioxidant 1076, and polyethylene wax according to a weight ratio of about 100 : 20 : 0.2 : 0.1 in a high speed ball grinder to prepare a mixture; extruding and granulating the mixture; blow molding the mixture to form a shell; and
in step c), immersing the shell in a chemical nickel plating solution for about 10 min again to form a first nickel layer with a thickness of about 3 µm; immersing the shell in a chemical copper plating solution for about 2 hours to form a copper layer with a thickness of about 10 µm on the first nickel layer; and immersing the shell in a chemical nickel plating solution for about 12 min again to form a second nickel layer with a thickness of about 4 µm on the copper layer; thus forming the plastic article as a shell for an electronic part of an automobile.

### Embodiment 5

The method in Embodiment 5 is substantially similar in all respects to that in Embodiment 1, with the exception of:
in step a), ball milling CuZrO₃ to form powders with an average diameter of about 900 nm; drying the powders; mixing PPO resin, CuZrO₃, calcium carbonate fiber, antioxidant 1076, and polyethylene wax according to a weight ratio of about 100 : 10 : 10 : 0.2 : 0.1 in a high speed ball grinder to prepare a mixture; extruding and granulating the mixture by a twin screw extruder; injection molding the mixture to form a shell; and
in step c), immersing the shell in a chemical nickel plating solution for about 8 min to form a nickel layer with a thickness of about 2 µm; immersing the shell in a chemical copper plating bath for about 4 hours to form a copper layer with a thickness of about 15 µm on the first nickel layer; immersing the shell in the chemical nickel plating solution for about 10 min again to form a second nickel layer with a thickness of about 3 µm on the copper layer; and strike plating or flash plating an aurum layer with a thickness of about 0.03 µm on the second nickel layer; thus forming the plastic article as a shell for an outdoor connector of a solar cell.

### Embodiment 6

A method for preparing a plastic article comprises the steps of:
a) mixing about 2.2 g of Na₂CO₃, about 98 g of CaCO₃, about 240 g of CuO, and about 330 g of TiO₂ powders uniformly; ball milling the powders in distilled water in a high speed ball grinder for about 12 hours to form a mixture; drying and calcining the mixture at a temperature of about 950°C for about 2 hours; ball milling the mixture again for about 4 hours; drying and granulating the mixture with PVA powders; pressing the mixture into circular sheets under a pressure of about 100 MPa; sintering the sheets at a temperature of about 1100°C for about 6 hours to form powders; ball milling the powders at a high speed until the average diameter of the powders reaches about 900 nm; analyzing the resulting product Na_{0.04}Ca_{0.98}Cu₃Ti₄O₁₂ by X-ray Photoelectron Specroscopy (XPS);
b) mixing PA6T resin, Na_{0.04}Ca_{0.98}Cu₃Ti₄O₁₂, antioxidant 1076, and polyethylene wax according to a weight ratio of about 100 : 10 : 0.2 : 0.1 to form a mixture; extruding and granulating the mixture; injection molding the mixture to form a shell;
c) patterning on the shell by a method substantially similar to that in step b) of Embodiment 1; and
d) the plating step is substantially similar in all respects to step c) of Embodiment 1, with the exception of: immersing the shell in a chemical nickel plating solution for about 8 min to form a nickel layer with a thickness of about 2 µm; immersing the shell in a chemical copper plating bath for about 4 h to form a copper layer with a thickness of about 15 µm on the first nickel layer; immersing the shell in the chemical nickel plating solution for about 10 min again to form a second nickel layer with a thickness of about 3 µm on the copper layer; and strike plating an aurum layer with a thickness of about 0.03 µm on the second nickel layer; thus forming the plastic article as a shell for an electric connector of an automobile engine.

### Embodiment 7

A method for preparing a plastic article comprises the steps of:
a) mixing about 3.3 g of La₂O₃, about 100 g of Ca₂CO₃, about 240 g of CuO, and about 330 g of TiO₂ powders uniformly; ball milling the powders in distilled water in a high speed ball grinder for about 12 hours to form a mixture; drying and calcining the mixture at a temperature of about 950°C for about 2 hours; ball milling the mixture again for about 4 hours; drying and granulating the mixture with PVA powders; pressing the mixture into circular sheets under a pressure of about 100 MPa; calcining the sheet at a temperature of about 1100°C for about 6 hours to form powders; milling the powders until the average diameter reaches about 1.0 µm; analyzing the resulting product Na_{0.01}Ca_{0.99}Cu₃Ti₄O₁₂ by XPS;
b) mixing PPS resin, Na_{0.01}Ca_{0.99}Cu₃Ti₄O₁₂, antioxidant 1076, and polyethylene wax according to a weight ratio of about 100 : 10 : 0.2 : 0.1 to form a mixture; extruding and granulating the mixture; injection molding the mixture to form a shell;
c) patterning on the shell by a method substantially similar to that in step b) of Embodiment 1; and
d) the plating step substantially similar in all respects to step c) of Embodiment 3 with the exception of: immersing the shell in a chemical copper plating solution for about 3 hours to form a copper layer with a thickness of about 12 µm; and immersing the support in a chemical nickel plating solution for about 10 min to form a nickel layer with a thickness of about 3 µm on the copper layer, thus forming the plastic article as a shell of an electric connector.

## Claims

1. A method for metalizing a plastic surface of a plastic article, the plastic article having at least a part thereof made from a support comprising a supporting material and a chemical plating promoter, wherein the chemical plating promoter is a perovskite-based compound represented by a general formula of ABO₃, in which A is one or more elements selected from groups 9, 10, and 11 of the periodic table and, optionally, one or more additional elements selected from groups 1, 2 and the lanthanide series of the periodic table, and B is one or more elements selected from groups 4 and 5 of the periodic table, the method comprising the steps of:
1) gasifying the plastic surface to expose the chemical plating promoter;
2) chemical plating a layer of copper or nickel on the plastic surface; and
3) plating the plated surface in step 2) by electroplating or chemical plating at least one more time to form a metalized layer on the plastic surface.

2. The method according to claim 1, wherein the plastic surface is gasified by laser to expose the chemical plating promoter.

3. The method according to claim 2, wherein the laser has a wavelength ranging from 157 nm to 10.6 µm with a scanning speed from 500 mm/s to 8000 mm/s, a scanning step from 3 µm to 9 µm, a scan time delay from 30 µs to 100 µs, a laser power from 3 W to 4W, a frequency from 30 KHz to 40 KHz and a filled distance from 10 µm to 50 µm.

4. The method according to claim 1, wherein the chemical plating promoter has an average diameter ranging from 20 nm to 100 µm.

5. The method according to claim 1, wherein the chemical plating promoter is selected from the group consisting of CaₓCU₄₋ₓTi₄O₁₂, Na_{0.04}Ca_{0.98}Cu₃Ti₄O₁₂, La_{0.}01Ca_{0.99}Cu₃Ti₄O₁₂, CuTiO₃, CuNiTi₂O₆, CuNbO₃, CuTaO₃ and CuZrO₃, where 0≤x≤4.

6. The method according to claim 1, wherein the support is a thermoplastic or a thermosetting resin, in which the thermoplastic includes a material selected from the group consisting of polyolefins, polycarbonates, polyesters, polyamides, polyaromatic ethers, polyester-imides, polycarbonate/acrylonitrile-butadiene-styrene composite, polyphenylene oxide, polyphenylene sulfide, polyimides, polysulfones, poly (ether ether ketone), polybenzimidazole, liquid crystalline polymer and any combination thereof; and the thermosetting resin includes a material selected from the group consisting of phenolic resin, urea-formaldehyde resin, melamine-formaldehyde resin, epoxy resin, alkyd resin, polyurethane and any combination thereof.

7. The method according to claim 1, wherein the chemical plating promoter amounts to 1 wt% to 40 wt%, based on the weight of the support.

8. The method according to claim 1, wherein the support further comprises a material selected from the group consisting of inorganic filler, antioxidant, light stabilizer, lubricant and any combination thereof.

9. The method according to claim 1, comprising the step of:
forming the plastic article with at least a part thereof made from the support comprising a supporting material and a chemical plating promoter.

10. The method according to claim 9, wherein the plastic article is formed by injection molding, blow molding, extruding or hot pressing.

11. The method according to claim 9, wherein the step 3) further comprises performing additional electroplating or/and chemical plating to form a Ni-Cu-Ni, Ni-Cu-Ni-Au, Cu-Ni, or Cu-Ni-Au layer on the support respectively.

12. The method according to claim 11, wherein the Ni layer has a thickness ranging from 0.1 µm to 50 µm, the Cu layer has a thickness ranging from 0.1 µm to 100 µm, and the Au layer has a thickness ranging from 0.01 µm to 10 µm respectively in the layers of Ni-Cu-Ni, Ni-Cu-Ni-Au, Cu-Ni and Cu-Ni-Au.

13. The method according to claim 9, wherein the chemical plating promoter is evenly distributed in the support.

14. A plastic article as manufactured by the method according to any one of claims 1 through 13.

## Patentansprüche

1. Verfahren zum Metallisieren einer Kunststofffläche eines Kunststoffartikels, wobei bei dem Kunststoffartikel mindestens ein Teil davon aus einem Träger hergestellt ist, der ein Trägermaterial und einen chemischen Plattierpromotor umfasst, wobei der chemische Plattierpromotor eine Verbindung auf Perowskitbasis ist, die durch eine allgemeine Formel von ABO₃ dargestellt ist, wobei A ein oder mehrere Elemente ausgewählt aus Gruppen 9, 10 und 11 der Periodentabelle und wahlweise ein oder mehrere zusätzliche Elemente ausgewählt aus den Gruppen 1, 2 und der Lanthanidserien der Periodentabelle ist und B ein oder mehrere Elemente ausgewählt aus den Gruppen 4 und 5 der Periodentabelle ist, wobei das Verfahren die Schritte umfasst des:
1) Vergasens der Kunststofffläche, um den chemischen Plattierpromotor bloßzulegen,
2) chemischen Plattierens einer Schicht Kupfer oder Nickel auf der Kunststofffläche; und
3) Plattierens der in Schritt 2) plattierten Fläche durch mindestens einmaliges Galvanisieren oder chemisches Plattieren, um eine metallisierte Schicht auf der Kunststofffläche zu bilden.

2. Verfahren nach Anspruch 1, wobei die Kunststofffläche durch Laser vergast wird, um den chemischen Plattierpromotor bloßzulegen.

3. Verfahren nach Anspruch 2, wobei der Laser eine Wellenlänge im Bereich von 157 nm bis 10,6 µm bei einer Scangeschwindigkeit von 500 mm/s bis 8000 mm/s, einem Scanschritt von 3 µm bis 9 µm, einer Scanzeitverzögerung von 30 µs bis 100 µs, einer Laserleistung von 3 W bis 4 W, einer Frequenz von 30 KHz bis 40 KHz und einem gefüllten Abstand von 10 µm bis 50 µm aufweist.

4. Verfahren nach Anspruch 1, wobei der chemische Plattierpromotor einen durchschnittlichen Durchmesser im Bereich von 20 nm bis 100 µm aufweist.

5. Verfahren nach Anspruch 1, wobei der chemische Plattierpromotor aus der Gruppe ausgewählt ist bestehend aus CaₓCu₄₋ₓTi₄O₁₂, Na_{0,04}Ca_{0,98}Cu₃Ti₄O₁₂, La_{0,01}Ca_{0,99}Cu₃Ti₄O₁₂, CuTiO₃, CuNiTi₂O₆, CuNbO₃, CuTaO₃ und CuZrO₃, wobei 0≤x<4.

6. Verfahren nach Anspruch 1, wobei der Träger ein thermoplastisches oder duroplastisches Harz ist, wobei das Thermoplast ein Material umfasst ausgewählt aus der Gruppe bestehend aus Polyolefinen, Polycarbonaten, Polyestern, Polyamiden, polyaromatischen Ethern, Polyesterimiden, Polycarbonat-/Acrylnitril-Butadien-Styrol-Verbundstoff, Polyphenylenoxid, Polyphenylensulfid, Polyimiden, Polysulfonen, Poly(etheretherketon), Polybenzimidazol, flüssigem kristallinem Polymer und irgendeiner Kombination davon; und das duroplastische Harz ein Material umfasst ausgewählt aus der Gruppe bestehend aus phenolischem Harz, Harnstoffformaledhyharz, Melaminformaldehydharz, Epoxidharz, Alkydharz, Polyurethan und Kombinationen davon.

7. Verfahren nach Anspruch 1, wobei der chemische Plattierpromotor 1 Gew.-% bis 4 Gew.-%, auf das Gewicht des Trägers bezogen, beträgt.

8. Verfahren nach Anspruch 1, wobei der Träger ferner ein Material umfasst ausgewählt aus der Gruppe bestehend aus anorganischem Füllstoff, Antioxidationsmittel, Lichtstabilisator, Gleitmittel und irgendeiner Kombination davon.

9. Verfahren nach Anspruch 1, umfassend den Schritt des:
Bildens eines Kunststoffartikels, wobei mindestens ein Teil davon aus dem Träger besteht, der ein Trägermaterial und einen chemischen Plattierpromotor umfasst.

10. Verfahren nach Anspruch 9, wobei der Kunststoffartikel durch Spritzgießen, Blasformen, Extrudieren oder Heißpressen gebildet wird.

11. Verfahren nach Anspruch 9, wobei der Schritt 3) ferner das Durchführen von zusätzlichem Galvanisieren und/oder chemischem Plattieren unter Bildung jeweils einer Ni-Cu-Ni-, Ni-Cu-Ni-Au-, Cu-Ni- oder Cu-Ni-AU-Schicht auf dem Träger umfasst.

12. Verfahren nach Anspruch 1, wobei die Ni-Schicht eine Dicke im Bereich von 0,1 µm bis 50 µm aufweist, die Cu-Schicht eine Dicke im Bereich von 0,1 µm bis 100 µm aufweist und die Au-Schicht eine Dicke im Bereich von 0,01 µm bis 10 µm in den Schichten von Ni-Cu-Ni, Ni-Cu-Ni-Au, Cu-Ni oder Cu-Ni-AU aufweist.

13. Verfahren nach Anspruch 9, wobei der chemische Plattierpromotor gleichmäßig in dem Träger verteilt ist.

14. Kunststoffartikel wie durch das Verfahren nach einem der Ansprüche 1 bis 13 hergestellt.

## Revendications

1. Procédé de métallisation d'une surface plastique d'un article en plastique, l'article en plastique ayant au moins une partie de celui-ci se composant d'un support comprenant un matériau de support et un promoteur de placage chimique, le promoteur de placage chimique étant un composé à base de pérovskite représenté par la formule générale ABO₃, dans laquelle A est un ou plusieurs éléments sélectionnés parmi les groupes 9, 10 et 11 du tableau périodique des éléments et, facultativement un ou plusieurs éléments supplémentaires sélectionnés dans les groupes 1, 2 et la série des lanthanides du tableau périodique des éléments, et B est un ou plusieurs éléments sélectionnés dans les groupes 4 et 5 du tableau périodique des éléments, le procédé comprenant les étapes consistant à :
1) gazéifier la surface plastique pour exposer le promoteur de placage chimique ;
2) plaquer chimiquement une couche de cuivre ou de nickel sur la surface plastique ; et
3) plaquer la surface plaquée de l'étape 2) par électroplacage ou placage chimique au moins encore une fois pour former une couche métallisée sur la surface plastique.

2. Procédé selon la revendication 1, dans lequel la surface plastique est gazéifiée par laser pour exposer le promoteur de placage chimique.

3. Procédé selon la revendication 2, dans lequel le laser a une longueur d'onde comprise dans la plage allant de 157 nm à 10,6 µm à une vitesse de balayage de 500 mm/s à 8000 mm/s, une étape de balayage de 3 µm à 9 µm, un retard de temps de balayage de 30 µs à 100 µs, une puissance laser de 3 W à 4 W, une fréquence de 30 KHz à 40 KHz et une distance remplie de 10 µm à 50 µm.

4. Procédé selon la revendication 1, dans lequel le promoteur de placage chimique a un diamètre moyen compris dans la plage allant de 20 nm à 100 µm.

5. Procédé selon la revendication 1, dans lequel le promoteur de placage chimique est sélectionné dans le groupe constitué par CaₓCu₄₋ₓTi₄O₁₂, Na_{0,04}Ca_{0,98}Cu₃Ti₄O₁₂, La_{0,01}Ca_{0,99}Cu₃Ti₄O₁₂, CuTiO₃, CuNiTi₂O₆, CuNbO₃, CuTaO₃ et CuZrO₃, où 0 ≤ x < 4.

6. Procédé selon la revendication 1, dans lequel le support est une résine thermoplastique ou thermodurcissable, dans lequel la résine thermoplastique comprend une substance sélectionnée dans le groupe constitué par les polyoléfines, les polycarbonates, les polyesters, les polyamides, les éthers polyaromatiques, les polyester-imides, un composite de polycarbonate/acrylonitrile-butadiène-styrène, un oxyde de polyphénylène, un sulfure de polyphénylène, les polyimides, les polysulfones, une poly(éther éther cétone), un polybenzimidazole, un polymère cristallin liquide et n'importe quelle combinaison de ceux-ci ; et la résine thermodurcissable comprend une substance sélectionnée dans le groupe constitué par une résine phénolique, une résine d'urée-formaldéhyde, une résine de mélamine-formaldéhyde, une résine époxy, une résine alkyde, un polyuréthane et n'importe quelle combinaison de ceux-ci.

7. Procédé selon la revendication 1, dans lequel le promoteur de placage chimique représente de 1 % en poids à 40 % en poids, par rapport au poids du support.

8. Procédé selon la revendication 1, dans lequel le support comprend en outre une substance sélectionnée dans le groupe constitué par une charge inorganique, un antioxydant, un stabilisateur de lumière, un lubrifiant et n'importe quelle combinaison de ceux-ci.

9. Procédé selon la revendication 1, comprenant l'étape consistant à :
former l'article plastique dont au moins une partie de celui-ci se compose du support comprenant un matériau de support et un promoteur de placage chimique.

10. Procédé selon la revendication 9, dans lequel l'article en plastique est formé par moulage par injection, moulage par gonflage, extrusion ou pressage à chaud.

11. Procédé selon la revendication 9, dans lequel l'étape 3) consiste en outre à réaliser un électroplacage et/ou un placage chimique supplémentaire pour former une couche de Ni-Cu-Ni, Ni-Cu-Ni-Au, Cu-Ni ou Cu-Ni-Au sur le support respectivement.

12. Procédé selon la revendication 11, dans lequel la couche de Ni a une épaisseur comprise dans la plage allant de 0,1 µm à 50 µm, la couche de Cu a une épaisseur comprise dans la plage allant de 0,1 µm à 100 µm, et la couche d'Au a une épaisseur comprise dans la plage allant de 0,01 µm à 10 µm respectivement dans les couches de Ni-Cu-Ni, Ni-Cu-Ni-Au, Cu-Ni et Cu-Ni-Au.

13. Procédé selon la revendication 9, dans lequel le promoteur de placage chimique est distribué uniformément dans le support.

14. Article en plastique manufacturé par le procédé selon l'une quelconque des revendications 1 à 13.
